

## UNITED STATES PATENT OFFICE

2,229,065

AUSTENITIC ALLOY STEEL AND ARTICLE  
MADE THEREFROMRussell Franks, Niagara Falls, N. Y., assignor to  
Electro Metallurgical Company, a corporation  
of West VirginiaNo Drawing. Application December 14, 1938,  
Serial No. 245,593

3 Claims. (Cl. 75—128)

The invention relates to austenitic chromium alloy steels and is particularly concerned with means for improving the hot working characteristics of such steels.

5 Chromium steels containing about 12% to 25% chromium, 6% to 20% of austenite-promoting metal of the group consisting of nickel, manganese, and mixtures thereof, and carbon in an amount not exceeding about 0.12%, are corrosion resistant, tough, and ductile. To improve 10 certain of the characteristics of these steels, for example, their resistance to intergranular corrosion, it has been proposed to add a substantial amount of one or more of the ferrite-promoting, 15 carbide-forming elements of the group consisting of titanium, zirconium, vanadium, columbium, tantalum, molybdenum and tungsten. While such elements effectively inhibit intergranular corrosion, their presence appears to 20 have a deleterious effect on the hot working characteristics of the steels. It is believed that the difficulties in hot working, usually manifest by tears, checks, or cracks in the steels, are caused by the partial decomposition of the austenite of the steel under the conditions of high 25 temperature and mechanical work, forming a small amount of an undesirable ferritic constituent throughout the austenite matrix. This small proportion of ferritic constituent appears to 30 detrimentally affect the hot workability of steels of the class in question.

Measures have been proposed to improve the hot working characteristics of such steels, but none has been entirely satisfactory. One proposal has been to increase the carbon content 35 and thus, by promoting a more stable austenite, to restrict both the tendency of the carbide-forming elements to form the undesirable ferritic constituent, and the tendency of the austenite 40 to decompose and form such a constituent during hot working. This expedient, while improving hot workability, has a deleterious effect, not only on the general corrosion resistance of the metal, but also on its resistance to intergranular 45 attack. It has also been proposed to promote a more stable austenite by increasing the nickel or manganese content, or combined nickel and manganese content of the steel above 20%, but this expedient is only partially effective and is more- 50 over, relatively expensive. The use of a very high proportion of nickel has the added disadvantage of increasing the hot-stiffness of the metal, thereby increasing the difficulty of working it.

55 I have found that the addition of relatively

small amounts of nitrogen to steels containing about 12% to 25% chromium, 6% to 20% of an austenite-promoting element of the group consisting of nickel, manganese, and mixtures thereof, carbon in an amount less than 0.12%, and a 5 total amount, not over 5%, of one or more of the ferrite-promoting, carbide-forming elements of the group consisting of titanium, zirconium, vanadium, columbium, tantalum, tungsten, molybdenum, and mixtures thereof considerably improves the hot working and other properties of such steels without impairing their excellent corrosion-resistance or without substantially increasing their resistance to deformation at hot working temperatures. The nitrogen content is 10 uniformly distributed throughout the steel and should be between 0.05% and 0.5%, preferably between 0.05% and 0.2%. As is customary in steels of this class, copper may be added in amounts up to about 2.5%. The maximum percentage of nitrogen that can be held in stable combination in these alloys depends on their chromium, nickel, and manganese contents. If the chromium content is 20% or over, and the nickel, manganese, or nickel-plus manganese content is low, the nitrogen content may rise to 15 0.5%, but when the chromium content is below 20%, and the nickel, manganese, or nickel-plus manganese content is high, it is advisable to keep the nitrogen content below 0.2%. 20

I have observed that the nitrogen imparts stability to the austenitic constituent of the steel, strengthens and otherwise improves the properties of the ferritic constituents particularly at elevated temperatures, and promotes a fine-grained structure throughout the steel. It is probable that these effects are responsible, at least in large part, for the improved hot workability of the steels and for the fact that during the heat treating of such steels the cooling rate necessary 35 for a given section, to retain a high proportion of austenite, can be slower than that necessary to retain the same proportion of austenite in a steel containing little or no nitrogen but otherwise of similar analysis. The reduced cooling 40 rate is particularly valuable in imparting good ductility and toughness to those articles, either cast or wrought, which, owing to their shape, thickness or other factors, could not be very rapidly cooled by known practical methods. 45

Another valuable characteristic resulting from the addition of nitrogen to the steels herein described is that the yield point and maximum strength of the hot-worked steels are increased substantially without the proportionate decrease 50

in impact strength and ductility which usually accompanies such improved properties.

This and other improvements in the physical properties of the hot-worked steels are indicated in the following table:

nitrogen, which counteracts the said adverse effect of the columbium; remainder iron and incidental impurities including not over 0.12% carbon.

2. Hot worked austenitic alloy steel containing 5

| No. | Composition (remainder Fe) |            |           |            |            |           | Tensile test results |       |            |            |      |       | 10 |
|-----|----------------------------|------------|-----------|------------|------------|-----------|----------------------|-------|------------|------------|------|-------|----|
|     | Percent Cr                 | Percent Ni | Percent C | Percent Cb | Percent Mo | Percent N | Y. P.                | M. S. | Percent EL | Percent RA | Izod | B. H. |    |
| 10  | 17.5                       | 9          | 0.07      | None       | None       | 0.04      | 34                   | 87    | 59         | 64         | 107  | 128   |    |
| 1   | 18.5                       | 9          | 0.09      | 1.1        | None       | 0.04      | 36                   | 90    | 54         | 70         | 101  | 140   |    |
| 2   | 18.0                       | 9          | 0.08      | 1.1        | None       | 0.11      | 48                   | 100   | 50         | 65         | 107  | 170   |    |
| 15  | 18.3                       | 10         | 0.06      | None       | 2.6        | 0.04      | 37                   | 90    | 57         | 73         | 98   | 146   | 15 |
| 4   | 18.3                       | 10         | 0.08      | None       | 2.6        | 0.10      | 42                   | 92    | 58         | 74         | 102  | 156   |    |
| 5   | 18.2                       | 9.6        | 0.06      | None       | 3.2        | 0.04      | 40                   | 92    | 54         | 73         | 97   | 163   |    |
| 6   | 18.2                       | 9.1        | 0.08      | None       | 3.2        | 0.13      | 49                   | 99    | 55         | 74         | 113  | 170   |    |
| 7   |                            |            |           |            |            |           |                      |       |            |            |      |       |    |

20 NOTE.—Steels No. 1 to 3 hot worked and water quenched from 1,150° C. before testing. Steels No. 4 to 7 hot worked and air cooled from 1,100° C. before testing.

20

In the above table, the following symbols are used: Y. P. for yield point in thousands of pounds per square inch; M. S. for maximum stress in thousands of pounds per square inch; per cent EL for percentage elongation in two inches in a standard 0.505 inch tensile sample; per cent RA for percentage reduction in area of cross section accompanying the elongation; Izod to designate the Izod impact resistance in foot pounds; and B. H. for the hardness on the Brinell scale.

The steels of the invention may be satisfactorily hot worked following the procedure ordinarily employed in working plain austenitic chromium 35 nickel steels. The resulting articles are free from the surface imperfections usually produced in hot worked austenitic chromium nickel steels containing ferrite-promoting, carbide-forming elements. Further, the improved hot working and 40 other characteristics of the steels herein described are obtained without deleteriously affecting the strength, toughness, ductility, or corrosion-resistance of the metal.

I claim:

45 1. Hot worked austenitic alloy steel containing between 12% and 25% chromium; between 6% and 20% nickel, a substantial proportion of the ferrite-promoting ingredient columbium, having a favorable effect on the corrosion resistance of the steel but an adverse effect on its hot working properties, but not exceeding 5%; 0.05% to 0.2%

between 12% and 25% chromium; between 6% and 20% nickel; substantial proportions of the ferrite - promoting ingredients columbium and molybdenum, having a favorable effect on the corrosion resistance of the steel but an adverse effect on its hot working properties, but not exceeding 5% in total sum; 0.05% to 0.2% nitrogen which counteracts the said adverse effect of the columbium and molybdenum; remainder iron and incidental impurities including not over 0.12% carbon.

25 3. Hot worked corrosion resistant austenitic alloy steel article containing between 12% and 25% chromium; between 6% and 20% of at least one material, promoting an austenitic structure, selected from the group consisting of nickel and manganese; a substantial proportion of at least one ferrite-promoting ingredient having a favorable effect on the corrosion resistance of the steel, but an adverse effect on its hot working properties, such ingredient or ingredients being in the aggregate not over 5% of the steel and being selected from the group consisting of titanium, zirconium, vanadium, columbium, tantalum, molybdenum, and tungsten; between 0.05% and 0.5% nitrogen which counteracts the said adverse effect of the ferrite-promoting ingredients; the remainder iron and incidental impurities including not over about 0.12% carbon.

40 45 RUSSELL FRANKS.

50